

July 27, 1937.

H. J. VAN ROYEN

2,088,282

PROCESS FOR THE PRODUCTION OF RAILS

Filed March 31, 1934

Fig.1



Fig. 1a



Fig. 2



Fig. 2a.



Fig. 3



Fig. 4



Inventor:

H. J. Van Royen

By: *Mark H. Clark*  
Atty's -

## UNITED STATES PATENT OFFICE

2,088,282

## PROCESS FOR THE PRODUCTION OF RAILS

Herman Johan van Royen, Hoerde, Germany

Application March 31, 1934, Serial No. 718,493  
In Germany April 10, 1933

7 Claims. (CL. 148—12)

This invention relates to an improvement in the manufacture of rails from a steel of eutectoid composition and of lamellar pearlitic structure as well as to the improved rails thus obtained.

- 5 Carbon steels containing about 0.9% of carbon and thus possessing the so-called eutectoid composition have the lamellar-pearlitic structure if they are protected from too rapid cooling after rolling. If said steels have an increased content 10 of manganese (more than 0.5%) or if they contain further so-called double carbide forming elements especially molybdenum, the steel must have a carbon content lower than 0.9% in order to maintain the eutectoid composition. For instance an unalloyed steel with 0.75% of manganese has the eutectoid composition with a carbon content of 0.75% and a molybdenum steel with 0.3% of molybdenum and 0.65% of manganese with a carbon content of 0.80%.
- 20 The present invention relates to a process for the treatment of steels with eutectoid composition and lamellar-pearlitic structure in which the carbon content lies below 0.9%, more particularly between about 0.65 and 0.80% and containing 25 manganese preferably between about 0.6 and 0.8% and molybdenum up to 0.3%. In addition thereto small amounts of the further double carbide forming elements chromium, tungsten, vanadium may be present singly or together. In 30 this case the manganese content may be decreased to about 0.5%.

The present invention aims at providing a process, the purpose of which is to impart to wear-resisting steels of the aforesaid composition and structure a further improvement of those mechanical properties, especially with regard to shock and impact stresses, which are important in practical use. According to the experience of the German State Railways, considerable importance must be attached in the case of steels with high resistance to wear and increased hardness to the requirement that said steels should behave just as well under the conditions of impact tests, as steels of lower hardness. In addition the reliable prevention of fractures under continuous stressing is a matter of the highest importance. These phenomena of fracture are attributable to the formation of hair cracks in the rail head and, consequently, if the formation of such cracks can 50 be reliably prevented, the prevention of fractures

under continuous stressing may be taken for granted.

It has been ascertained in accordance with the present invention that an important improvement can be obtained, in relation to the aforesaid two requirements, by the maintenance of definite temperature conditions in rolling the steel so that when the temperature has fallen to about 1000° C. in the penultimate pass, the rolling is not continued immediately, the material being, on the contrary, allowed to cool until its temperature has fallen to a little above 900° C. and then continuing rolling in the final pass at that temperature, in which event the end temperature will be slightly below 900° C. 15

This method of working is suitably performed by starting with comparatively small ingots which are first allowed to cool gradually and then slowly re-heated before rolling. The ingots should weigh about 2 to 2.5 tons. The slow cooling can 20 be effected by allowing the ingots to remain longer than usual in the moulds, and consequently for about 5 hours, instead of the usual period of two hours.

According to the present invention, therefore, 25 the rolling is carried out by casting the steel in small ingots which, before being worked, are left to cool slowly, and are then reheated to the temperature required for rolling. The cooling should preferably be continued until room temperature 30 is reached. After the second pass the temperature is about 1180° C. and after the last pass but one, about 1000—1050° C. After the penultimate pass the material is allowed to cool down to 910—900° C. and is then put through the final pass, 35 so that its temperature descends through the 900° C. level during that operation. It has also been found advisable to make arrangements so that the rail, which in the ordinary method of treatment bends considerably on the cooling bed, 40 and has to be subjected to extensive deformation in cold straightening, is already substantially straightened on the cooling bed. For this purpose the rail, after leaving the rolls, and therefore in a warm state, is subjected to a preliminary bending of such a character as to be counter, in direction and extent, to that experienced by the rail in cooling. Under this treatment, the steel leaves the cooling bed in a nearly straight 45 condition so that its shape requires to be only 50

slightly modified afterwards. This treatment also contributes to furnishing a product of maximum reliability.

This feature of the present invention is illustrated by way of example with reference to the accompanying drawing in which

Fig. 1 is a side view showing the curved condition of a rail after normal treatment.

Fig. 1<sup>a</sup> is a transverse section of the rail.

Fig. 2 illustrates in which manner the rail is preliminarily bent according to the invention.

Fig. 2<sup>a</sup> is a transverse section of the rail shown in Fig. 2.

Figs. 3 and 4 are side views of rails subjected to impact tests.

In order to obtain the finished rail in nearly straight condition the rail is subjected to a preliminary bending contrary to the deformation otherwise occurring in the rails.

In order not to disturb the development of the lamellar-pearlitic structure of the steel while cooling the steel must be protected against excessive loss of heat, in known manner. With this object the steel is not cooled on the cooling bed in the usual manner, but is inserted at about 750° C. under an insulated hood, and left to cool therein to about 500° C. whereupon it can be further cooled in the air.

According to the facts I have ascertained, the prevention of the cracks is not attributable to the retarded cooling which, on the contrary, serves merely to ensure the development of the lamellar-pearlitic structure. The dangerous transverse cracks do not appear even when the specified measures for retarding the cooling are omitted.

The following is a preferred composition of the steel: Carbon 0.73-0.80%, manganese 0.80-0.65%, molybdenum 0.3-0.2%. 0.15% may be taken as the minimum content of molybdenum from which an effect in the sense of the invention can be expected. The molybdenum may be entirely or partially replaced by chromium, tungsten or vanadium, in which event the manganese content can be reduced to about 0.5%. In any case, however, care must be taken to preserve the eutectoid structure. Therefore the following upper limits are to be observed:

|    | Percent              |  |  |  |  |  |  |  |  |
|----|----------------------|--|--|--|--|--|--|--|--|
| 50 | Chromium up to about |  |  |  |  |  |  |  |  |
|    | 0.5                  |  |  |  |  |  |  |  |  |
|    | Tungsten up to about |  |  |  |  |  |  |  |  |
|    | 0.7                  |  |  |  |  |  |  |  |  |
|    | Vanadium up to about |  |  |  |  |  |  |  |  |
|    | 0.2                  |  |  |  |  |  |  |  |  |

For instance favourable results were obtained with steels of the following composition

| C       | Mn      | Mo      | Cr      | W       | V       |                             |
|---------|---------|---------|---------|---------|---------|-----------------------------|
| Percent | Percent | Percent | Percent | Percent | Percent |                             |
| 0.72    | 0.65    | 0.27    | 0.40    |         |         |                             |
| 0.68    | 0.68    | 0.30    | 0.47    |         |         |                             |
| 0.75    | 0.68    | 0.20    | 0.30    | 0.35    | 0.20    | Balance substantially iron. |
| 0.78    | 0.75    | 0.15    |         | 0.70    |         |                             |

The secondary components, such as silicon, phosphorus and sulphur are present to the same extent as usual in rails. That is to say the silicon content may amount to about 0.2 to 0.3% and the content of phosphorus and sulphur to below 0.04%.

The preferred properties possessed by the rails produced by the process of the present invention by comparison with such rails made from eutectoid steels with an increased content of manganese, manganese and chromium, or manganese and molybdenum without, however, being sub-

jected to the treatment of the present invention can be gathered from the appended table.

The molybdenum steel treated in accordance with the process of the present invention is considerably superior to the other wear-resisting 5 steels with eutectoid structure in point of resistance to impact. Moreover, as already mentioned, it has no tendency to form cracks and consequently offers a greater resistance to continuous stressing. 10

#### Impact test on rails S 49

First blow 5000 mkg., each additional 3000 mkg. Weight of hammer 1000 kg., prescribed bend 80 mm. 15

| Method of manufacture of the rails                                                          | Type of wear-resisting steel                                                                                                                | Mean deflection prior to fracture mm. |
|---------------------------------------------------------------------------------------------|---------------------------------------------------------------------------------------------------------------------------------------------|---------------------------------------|
| Ordinary.....                                                                               | Eutectoid carbon steel with 0.75-0.80% of C. and 0.80-0.70% Mn. Eutectoid steel with 0.70-0.75% of C., 0.65-0.50% of Mn and 0.4-0.5% of Cr. | 84 20                                 |
| Normal Mo steel with eutectoid structure.                                                   | Eutectoid steel with 0.73-0.80% of C., 0.80-0.65% of Mn and 0.3-0.2% of Mo. do.....                                                         | 87 95 25                              |
| Steel of same composition, treated in accordance with the process of the present invention. |                                                                                                                                             | 110 30                                |

The manner in which the invention may be carried into practice is more particularly illustrated by the following examples: 35

From melts of the following composition:

| Melt   | C %  | Mn % | P %   | Si % | S %   | Cr % | Cu %  | Mo % |
|--------|------|------|-------|------|-------|------|-------|------|
| A..... | 0.78 | 0.76 | 0.030 | 0.28 | 0.023 | 0.08 | 0.18  | 0.22 |
| B..... | 0.80 | 0.67 | 0.038 | 0.29 | 0.021 | 0.07 | ..... | 0.22 |
| C..... | 0.75 | 0.74 | 0.034 | 0.28 | 0.018 | 0.06 | ..... | 0.25 |
| D..... | 0.78 | 0.70 | 0.031 | 0.30 | 0.022 | 0.05 | ..... | 0.17 |

Ingots of a weight of 2480 kg. were cast. They 45 were cooled after casting to ordinary temperature and inserted into a skid-furnace in the cold state. Herein they were heated to the temperature required for rolling of about 1200 to 1250° C. Thereupon they were rolled into rails of the profile 50 called "S 49". During the rolling treatment the following rolling temperatures were observed:

| Melt   | After the second pass | After the penultimate pass |     |
|--------|-----------------------|----------------------------|-----|
|        |                       | °C.                        | °C. |
| A..... | 1170                  | 990                        |     |
| B..... | 1180                  | 1010                       |     |
| C..... | 1180                  | 1020                       |     |
| D..... | 1190                  | 1010                       | 60  |

Thereupon the rails were left to cool down to about 900° C. and passed the final calibre at this temperature.

From each rolling length two rails of 15 meters 65 were cut. On the cooling bed said rails were bent through over the foot. By a preliminary bending of about 500 mm. it could be obtained that they were almost straight when the cooling was complete. After the preliminary bending the rails passed an isolated hood. The travelling time amounted to about half an hour. When leaving the hood they were found to have a temperature between about 500 and 520° C. 70 75

*Results of impact tests*

The impact tests were carried out after the prescriptions of the German State Railways. First blow 5000 mkg., each additional, 3000 mkg. Weight of hammer 1000 kg., prescribed bend 80 mm.

| 10 | Melt | Mean deflection mm. |
|----|------|---------------------|
| A  |      | 109                 |
| B  |      | 105                 |
| C  |      | 113                 |
| D  |      | 102                 |

The improved rail obtained in accordance with my invention is distinguished from rails of the same composition which have been rolled in ordinary manner by being free from cracks and possessing a substantially higher deflection, as illustrated by the foregoing examples. The mean deflection obtained under impact stresses is furthermore illustrated by reference to the accompanying drawing in which

Fig. 3 shows a rail the head of which has been subjected to the impact test prescribed by the German State Railways, the conditions of which are above referred to. The test was interrupted after 10 blows, the deflection amounted to 156 mm.

Fig. 4 shows a rail the foot of which has been subjected to an impact test under the same conditions above referred to. The foot received 8 blows and had a deflection of 110 mm.

It may be remarked that the method above described may be altered in various respects without departing from the spirit of my invention. Thus it is, of course, possible to obtain the lamellar-pearlitic structure in the rolled articles by cooling them in a covered or non-covered excavation or pit or by retarding the cooling in any other manner. Such details in the performance of my invention are, of course, quite familiar to those skilled in the art.

What I claim and desire to secure by Letters Patent of the United States is:

1. A process for the production of rails by rolling from a steel containing between about 0.65 and 0.80% of carbon, between about 0.5 and 0.8% of manganese and between about 0.15 and 0.3% of molybdenum, which comprises cooling the work to a temperature somewhat above 900° C. prior to the final pass so that it leaves the final pass with a temperature below about 900° C.

2. A process for the production of rails by rolling from a steel containing between about 0.65 and 0.80% of carbon, between about 0.5 and 0.8% of manganese and between about 0.15 and 0.3% of molybdenum in which small ingots of a weight of about 2 to 2.5 tons of said steel are subjected to a rolling treatment in which the work is cooled to a temperature somewhat above 900° C. prior to the final pass so that it leaves the final pass with a temperature below 900° C.

3. A process for the production of rails by rolling from a steel containing between about 0.65 and 0.80% of carbon, between about 0.5 and 0.8% of manganese and between about 0.15 and 0.3% of molybdenum which comprises casting small ingots of a weight of about 2 to 2.5

tons from said steel, cooling said ingots to ordinary temperature, reheating them to the temperature required for rolling and finally rolling them into rails of the desired shape, cooling the work to a temperature somewhat above 900° C. during the rolling prior to the final pass so that it leaves the final pass with a temperature below about 900° C.

4. A process for the production of rails by rolling from a steel containing between about 0.65 and 0.80% of carbon, between about 0.5 and 0.8% of manganese and between about 0.15 and 0.3% of molybdenum which comprises casting small ingots of a weight of about 2 to 2.5 tons from said steel, cooling said ingots to ordinary temperature, reheating them to the temperature required for rolling and finally rolling them into rails of the desired shape, cooling the work to a temperature somewhat above 900° C. during the rolling prior to the final pass so that it leaves the final pass with a temperature below about 900° C., thereafter subjecting the rail to a preliminary bending, counteracting the bending stresses occurring after cooling and finally retarding cooling of the rail on the cooling bed so that the development of the lamellar-pearlitic structure is preserved.

5. A process for the production of rails by rolling from a steel containing between about 0.73 and 0.80% of carbon, between about 0.80 and 0.65% of manganese and between about 0.3 and 0.2% of molybdenum in which small ingots of a weight of about 2 to 2.5 tons of said steel are subjected to a rolling treatment in which the work is cooled to a temperature somewhat above 900° C. prior to the final pass so that it leaves the final pass with a temperature below 900° C.

6. A process for the production of rails by rolling from a steel containing between about 0.73 and 0.80% of carbon, between about 0.80 and 0.65% of manganese and between about 0.3 and 0.2% of molybdenum which comprises casting small ingots of a weight of about 2 to 2.5 tons from said steel, cooling said ingots to ordinary temperature, reheating them to the temperature required for rolling and finally rolling them into rails of the desired shape, cooling the work to a temperature somewhat above 900° C. during the rolling prior to the final pass so that it leaves the final pass with a temperature below about 900° C.

7. A process for the production of rails by rolling from a steel containing between about 0.73 and 0.80% of carbon, between about 0.80 and 0.65% of manganese, and between about 0.3 and 0.2% of molybdenum which comprises casting small ingots of a weight of about 2 to 2.5 tons from said steel, cooling said ingots to ordinary temperature, reheating them to the temperature required for rolling and finally rolling them into rails of the desired shape, cooling the work to a temperature somewhat above 900° C. during the rolling prior to the final pass, so that it leaves the final pass with a temperature below about 900° C., thereafter subjecting the rail to a preliminary bending counteracting the bending stresses occurring after cooling and finally retarding the cooling of the rail on the cooling bed so that the development of the lamellar-pearlitic structure is preserved.